

# UNITED STATES PATENT OFFICE.

EMIL KANET, OF AGRAM, HUNGARY, ASSIGNOR, BY MESNE ASSIGNMENTS, TO THE CHEMICAL FOUNDATION, INC., A CORPORATION OF DELAWARE.

## METHOD OF DRESSING HIDES.

1,367,054.

Specification of Letters Patent. Patented Feb. 1, 1921.

No Drawing.

Application filed June 28, 1916. Serial No. 106,524.

To all whom it may concern:

Be it known that I, EMIL KANET, a subject of the Emperor of Austria, King of Hungary, residing at Agram, Hungary, 5 have invented a certain new and useful Method of Dressing Hides, of which the following is a full, clear, and exact specification.

My invention relates to a method of dressing hides by means of hydrolytically split 10 tanning-solutions.

It is well known that through the application of heat several salts precipitate from their aqueous, hydrolytically split solutions, 15 basic heavy soluble salts hydroxids and ox- 20 nids. The presence of an electrolyte will stabilize the colloidal solution of the tanning agent.

Such salts have tanning qualities which 25 in acidic solutions act more slowly than in basic ones, as far as they have tanning qualities at all.

My invention is based on the fact that solutions of the same basicity tan more slowly 30 or more weakly at relatively low temperatures, *i. e.* 0°-10° C. I am going to exemplify both of these cases in the following paragraphs of this specification design- 35 nated by the letters *a* and *b*.

30 *a.* The results obtained in the tannery by using strong chromic oxid subsalts and by using organic compounds of chromic oxid at least in diluted solutions are very doubtful, for such solutions are not stable and 35 hence precipitate chromic oxid upon standing, which oxid becomes distributed over the surface of the hide and is only very poorly absorbed thereby.

But I have found that if these solutions 40 are cooled, then they remain clear even if they are not used for a long time. In other words, the solutions are stable under these conditions.

Such a cooled solution tans the hide well, 45 slowly and uniformly and thus a strong basic solution or an organic compound of chromic oxid may be employed which makes the leather full and soft.

The same good results are obtained when 50 using ferric salts and aluminum salts, in the same manner.

With ferric salts another advantage is obtained by my method: It is well known,

that organic substances become better oxidized by iron-solutions, the higher their 55 temperature is and the more acid has been used.

Heretofore the solutions were generally made basic to a certain degree only, as otherwise ferric hydrate precipitates too 60 readily and retards the tanning operation and the surface of the hide becomes over-tanned and hard.

Moreover such a solution oxidizes the 65 fibers of the hide and weakens it.

In contradistinction thereto, if according to my present invention such a solution is allowed to cool off, it will be possible to make it basic to a high degree, without running in danger of bad tanning and the 70 fibers of the hide is not weakened.

*b.* If a solution is acidified to such a degree, that it forms a leather-curing compound at relatively low temperatures, for example at 0°-10° C., and if hereupon the 75 hide is caused to absorb the said solution, then, after subsequent heating, the absorbed solution tans the hide well and quickly.

Example:

According to my present invention I place 80 the hide into a solution of ferric acetate, in which advantageously sodium chlorid or another electrolyte, for example sodium acetate is dissolved. A solution containing from  $\frac{1}{2}$  to  $2\frac{1}{2}$  %  $Fe_2O_3$  corresponding to a 85 solution having a strength of about one to five per cent. of ferric acetate gives the best results. The hide is left in the tanning liquor for a sufficient length of time until, according to trial and experience, it has 90 absorbed a sufficient amount of the tanning liquor, is removed from the solution and placed into a warm (for example from 45° to 50° C.) weak solution of salt, or it may be suspended within a warm room. The 95 tanning-liquor, absorbed by the hide becomes active soon after the hide has been exposed to heat for about a minute. Hereafter the hide is stored for a short time during which the ferric oxid becomes chemically combined with the hide substance.

If together with the tanning solution filling materials are introduced into the hide (for example flour), then these materials become fixed in the same by the precipita- 105 tion of the basic radical of the iron acetate.

The tanning of leather by impregnating the same with a solution of a chromium salt and thereafter raising the temperature of the impregnated hides, is a well known process.

One of the essential features of my method, distinguishing the same from the known methods, is to be seen in the fact that my method is a so-called one bath 10 method, while the methods heretofore known constitute a so-called "double bath" method.

According to the present invention it is possible to use a single tanning salt either 15 separated or several of such salts together, in both instances, (and at the end of the tanning process) at a reduced temperature, and it is also possible to operate by using at the beginning a relatively low temperature 20 and subsequently heating.

By this process excellent result can be achieved, if ferric salts predominate and only small portions of chromic oxid or chromic salts are used.

25 My invention therefore presents a rapid

and cheap tanning method by means of which an excellent product is obtained.

What I claim is:

1. A method of treating hides which consists in tanning the hides by immersing 30 them into basic solutions of metallic salts in their higher oxid state in the presence of an electrolyte and at a low temperature and heating the wet hide for separating the basic oxids of the salts upon and between 35 the hide fibers.

2. A method of treating hides which consists in tanning the hides by immersing them into a solution of ferric acetate in the presence of sodium chlorid, at a low temperature and heating the wet hide for separating the basic oxids of the salts upon and 40 between the hide fibers.

In testimony whereof I affix my signature in presence of two witnesses.

EMIL KANET.

Witnesses:

MORIZ GELBHUN,  
AUGUST FUGGER.